

Jan. 1, 1935.

W. J. KELLY

1,986,401

PROCESS FOR CARBON STRUCTURE CONTROL IN IRON

Filed Dec. 19, 1930



INVENTOR.

WILLIAM J. KELLY.

BY *Hugo A. Maerlender*

ATTORNEY.

## UNITED STATES PATENT OFFICE

1,986,401

PROCESS FOR CARBON STRUCTURE  
CONTROL IN IRON

William J. Kelly, Elkins, W. Va.

Application December 19, 1930, Serial No. 503,457

3 Claims. (Cl. 148—3)

The presence of carbon in iron and alloys thereof results in widely varying metallic structures in the castings produced. The characteristics of strength, hardness, density, heat resistance, and resistance to wear, shock, stresses and the like are all directly dependent in part on the condition in which the alloyed carbon exists in the metal.

This invention relates generally to the structure of carbon in its various forms and alloys with iron. It provides a practical and efficient method for controlling the combined and graphitic carbon contents and permitting any desired percentages of these two elements in manufacturing iron castings for a wide variety of purposes.

In particular it relates to a process of heat treatment for iron castings and especially with the purpose of controlling the carbon form and its manner of association in the resulting metallic structure. A specific application of my invention is the manufacture of plunger castings for making glass tumblers and the like.

The primary object of the invention resides in the production of castings for a wide variety of purposes by controlling the heating and cooling in relation to the time involved in either of these processes and also relative to the carbon states and content in the alloy. A further object is to provide an accurate control of the heating and the manner and rate of cooling of the castings for the purpose of controlling the carbon structure.

As a preliminary step to the treatment herein-after described a casting is made in the form in which the metal is to be finally used and of proportions as are presently to be explained. Various purposes necessitate different quantities of the elements entering into the alloy as well as quantities of added elements including chromium, vanadium and nickel or combinations thereof, also titanium, tungsten and molybdenum.

In general the constituents of the alloy are those essential to the production of white iron and the constituents will vary in the following limits: carbon from 3.00 to 4.00 per cent; silicon .5 to 1.00 per cent; manganese .70 to 1.50 per cent; phosphorus 0 to .20 per cent and sulphur 0 to .10 per cent. In general the carbon in the castings is in the form of cementite or in solid solution. The combined condition of the carbon is readily attained.

As distinguished from the heat treatment of ordinary gray cast iron in which only .9 per cent

of the carbon content of the iron is taken into consideration for treatment under this invention carbon is formed in one condition alone, and then by a heat treatment at high temperatures the uniform carbon compound is decomposed in free or temper carbon and the subsequent control of the temperature determines the condition in which the carbon reenters into combination with the iron. Where carbon exists in the castings in two forms above the critical range a portion of the free carbon enters solid solution and slow cooling through the critical range allows the carbon to produce the pearlitic structure. Below the critical range the finished product consists of ferrite and cementite plus mechanically mixed carbon in the form of graphite. Where all of the carbon is formed in solid solution in the castings, the heat treatment precipitates a quantity of temper carbon and slow cooling through the critical range permits the remainder of the carbon to combine with the iron and form cementite. In either case the results are identical and the treatment is applicable to all classes of castings irrespective of the carbon condition.

The metal for the casting to be treated may be melted either in a cupola, air or open hearth furnaces or electric furnace and may be poured into sand molds provided the iron mixture is suitable and the section of the casting light, or of such thickness that the rate of cooling through the freezing or setting point of the metal will be sufficiently rapid to produce castings in which substantially all of the carbon is in solid solution. For castings of heavier section it is necessary to pour the metal into iron chill or permanent molds so that the cooling rate will be extremely rapid through the freezing period and the resulting castings white.

Since only a portion of this invention admits of illustration a special form of such a casting is illustrated in the annexed drawing in which

The figure is a side elevation of a completed casting specially adapted for use by the process hereinafter described.

For convenience of illustration the casting 1 represents a plunger casting for making glass tumblers whose physical requirements of close grain density, high machinable hardness, high resistance to heat and oxidation and freedom from scaling has thus been prepared. When the casting 1 is removed from the mold its outer surface is black and in this condition the casting is removed to a furnace for treatment. In the case of the plunger castings hereinafter specially

described, the castings are given an immersion in milk of lime to protect the outer surfaces.

Any type of furnace is adequate for the heat treatment to which the casting is subject but the appropriateness of the furnace to the shape of the casting should be observed in its construction. Adequate control of the temperatures to be attained is a requisite of the process as well as the provision of means for observing the temperatures. For this latter purpose an indicating pyrometer is preferably employed.

The control of the combined carbon in the iron casting is the result of the two elements of temperature and time and depends on a carbon condition which may be readily controlled. Temperatures up to 1300° F. do not materially affect the iron carbide of white chilled cast iron but I have found that with increasing temperatures the rate of the carbon precipitation becomes very rapid until at 1750° F. the rate is very rapid and breaks down the combined carbon content to a percentage which will enable the casting to be machined. The furnace in which the casting is treated should be able for this reason to attain temperatures of 2000° F. and above.

The temperature is gradually raised requiring from 40 to 45 minutes to approximately 1750 degrees. It is maintained at this temperature for about fifteen minutes and then allowed to cool in the furnace to approximately 1250° F. in the same gradual manner substantially as the temperature was raised. Various modifications in the treatment can be made depending upon the section and weight of the castings which are being treated; in general, thin castings require a shorter treatment than heavier ones. In this manner castings may be produced whose hardness may vary from 800 Brinell to 100 Brinell.

The treatment is, of course, not limited to slow cooling and I have found that iron castings prepared as in this process may be quenched from temperatures of 1700° F. to 1100° F. With such treatment temperatures above the critical temperature, or approximately 1300° F. produce hardness while below the hardness of the annealed samples is unaltered. Iron hardened in this manner may be restored to its normal state before tempering by heating to the critical temperature and permitting it to cool slowly. While similar treatment administered to ordinary gray iron produces hardening, iron produced by this process responds more readily and in a greater degree.

A semi-malleable product may be produced by maintaining the castings at a high temperature for three or four hours and then allowing them to cool to 1100 or 1200° F., at which temperature they are maintained for approximately two hours. For such treatment the castings are placed in annealing boxes and surrounded with charcoal or lime. The iron thus produced is more ductile, tougher and its tensile and transverse strengths are improved.

For special purposes, as suggested, various alloys are formed to effect the desired result in combination with the carbon. Under this manner of treatment I have found castings of the following analyses unsuited for plunger castings such as are used in casting glassware but satisfactory for abrasive resisting castings for valve seats and the like.

Silicon .9 to 1.00, sulphur .144-.154, phosphorus .36 to .28, manganese .59 to .95; chro-

mium .16 to .30, nickel .08 to .25, graphitic carbon 2.83 to 1.70 and combined carbon .87 to 2.11. Nevertheless, an alloy comprising .90 silicon; sulphur .07, phosphorus .07 to .10, manganese .73, chromium .16, nickel .10, and 3.60 carbon, is admirably suited for treatment by this process to produce plunger castings. The low sulphur and phosphorus content insures high heat resisting qualities. Chromium in this amount produces a double carbide of iron and chromium which does not break down in the least under exposure to the relatively high temperatures to which the casting is subjected during treatment, while the nickel assists in producing a fine grain throughout the casting. Small percentages of nickel are more suitable for this purpose, I have found, than larger quantities. The percentages of silicon and carbon are proportioned to produce in the iron a strong hard chill with a high combined carbon content insuring a minimum of shrinkage upon solidification and thereby avoiding disintegrating tendencies under heat characteristic of irons having high coefficients of expansion.

However, I do not desire to be limited to the specific analyses outlined for specific purposes since the process is applicable to all metals within the limits previously suggested including substantially all types of iron castings. In all cases, it is the percentages and distribution of the combined and graphitic carbon which are of importance. The carbon content made uniform and homogeneous throughout all areas of the casting by this process insures homogeneity of physical characteristics of strength, hardness, grain density, heat resistance, resistance to wear, shock, stresses and the like.

Cast iron made and treated by this process, I have found, has improved physical qualities and iron castings can be manufactured having a much higher machinable hardness than castings made by other methods. It should be obvious that the graphitization process can produce castings in addition to the purposes noted which are adaptable as gears, rolls, chemical castings and machine and automobile castings.

Having thus described my invention what I claim as new and desire to secure by Letters Patent is:

1. The process of carbon control in iron castings which consists in pouring metal having a carbon content substantially from 3.00 to 4.00 per cent, in a chill mold, reheating the casting in a maximum period of approximately forty-five minutes to approximately 1750° F., maintaining the casting at this temperature for a maximum period of fifteen minutes, cooling the casting through a maximum period of approximately forty-five minutes to approximately 1250° F. and cooling the casting further to room temperature.

2. The process of carbon control in iron castings adaptable as plungers and the like which consists in pouring metal comprising substantially .90 per cent silicon, .07 per cent sulphur, .07 to .10 per cent phosphorus, .7 per cent manganese, .16 per cent chromium, .10 per cent nickel and 3.60 per cent carbon into a chill mold, covering the casting with a protective coating, slowly reheating the casting to approximately 1750° F., maintaining the casting at this temperature for a short time and permitting the casting to cool slowly substantially as it was heated.

3. The process of carbon control in iron cast-

ings adaptable as plungers and the like which consists in pouring metal comprising substantially .90 per cent silicon, .07 per cent sulphur, .07 to 1.00 per cent chromium, .10 per cent nickel and 3.60 per cent carbon into a chill mold covering the casting with a protective coating, slowly reheating the casting over a period of substan-

tially forty-five minutes to approximately 1750° F., maintaining the temperature for approximately fifteen minutes, permitting the casting to cool to approximately 1250° F. throughout a like period of approximately forty-five minutes, and further cooling the casting to room temperature.

WILLIAM J. KELLY.